

## UNITED STATES PATENT OFFICE.

FERNANDO SOMOZA VIVAS, OF OAKLAND, CALIFORNIA, ASSIGNOR OF ONE-HALF TO  
WILLIAM M. STEELE, OF SAN FRANCISCO, CALIFORNIA.

## FIREPROOF ROOFING MATERIAL.

No Drawing.

Application filed June 14, 1923. Serial No. 645,351.

The invention relates to a roofing material commonly known as roof tar and has as an object the provision of a material of this nature which will be non-inflammable. A further object of the invention is the provision of material of this nature which will be cheap to produce and which will efficiently perform the usual function of material of this nature at the same time rendering the roof fire proof.

The formula which it is preferred to use as a physical embodiment of the invention comprises the following ingredients in the proportions named:

|                   | Parts |
|-------------------|-------|
| 15 Asphalt        | 40    |
| Rosin             | 10    |
| Drying oil        | 15    |
| Wood charcoal     | 10    |
| 20 Borax          | 12½   |
| Ammonium sulphate | 12½   |

The wood charcoal must of course be used in powdered form. Instead of the asphalt other bitumens may be used as for instance 25 gilsonite. The material prepared by the above formula may be used in the ordinary manner in the laying of roofs and has the

advantage not only of rendering the roof non-inflammable, thereby protecting the building upon which it is used from fire, 30 but it will reduce the fire hazards of the places where it is stored. If desired the material may be made an ingredient of the "prepared roofing" made of asphalt and felt which is in common use thereby rendering 35 the same fire proof.

Minor changes may be made in the proportion of parts and known equivalents may be substituted for some of the ingredients named without departing from the spirit 40 of the invention.

I claim:

1. A fire proof roofing material, comprising, in combination, asphalt, rosin, linseed oil, powdered charcoal, borax, ammonium sulphate, in proportions to produce a fire-proof roofing material.

2. A fire proof roofing material, comprising, in combination, asphalt 40 parts, rosin 10 parts, drying oil 15 parts, wood charcoal 10 parts, borax 12½ parts, ammonium sulphate 12½ parts.

FERNANDO SOMOZA VIVAS.